

## UNITED STATES PATENT OFFICE

2,356,367

## HIGH TEMPERATURE LUBRICANT

Donald L. Wright, Westfield, N. J., assignor, by  
mesne assignments, to Jasco, Incorporated, a  
corporation of Louisiana

No Drawing. Application November 22, 1940,  
Serial No. 366,714

14 Claims. (Cl. 252—29)

This invention relates to a lubricating composition and to methods of lubrication, and more particularly to those suitable at high temperatures, especially at temperatures high enough to cause charring or varnish and tar formation with the lubricating oil compositions used heretofore.

One object of the invention is the lubrication of devices such as oven conveyor chains, wheel bearings of kiln cars, annealing oven cars, ejector pins and other hot moving parts of die-casting machines, etc., which are required to operate at extremely high temperatures, i. e., above about 400° F., as, for instance, 500° F., 1,000° F., or higher. When conventional lubricating oils or greases are subjected to such hot operating conditions, decomposition of the petroleum ingredient eventually occurs, with the formation of end products which are hard, abrasive, carbonaceous or coke-like materials which reduce clearance between rubbing members and tend to promote wear.

Broadly, this invention comprises a method of lubricating metal surfaces which in the absence of a lubricant would move in contact with each other at temperatures above about 400° F., by applying to said contacting surfaces a lubricant comprising a major proportion of a volatile solvent such as a light hydrocarbon oil, having a final boiling point below 750° F. and having a viscosity below about 45 seconds Saybolt at 100° F., said oil containing dissolved therein a thickener such as a viscosity-increasing saturated linear aliphatic, preferably hydrocarbon polymer having a molecular weight above about 800 and having the property, when heated to high temperatures, e. g. above 400° F., of depolymerizing without formation of tar and coke, the amount of said polymer being sufficient to make a solution having a viscosity of at least 100 seconds Saybolt at 100° F.

According to another aspect of the invention, there may also be added to the lubricants described above a small amount of a non-abrasive solid which is non-combustible at temperatures up to 2500° F., the particles of which have a smooth surface suitable for solid lubrication. Such materials include graphite, mica, etc., the preferred substance being colloidal graphite, because it is substantially pure, i. e., containing not more than about 0.02% of ash. This colloidal graphite is preferably added in the form of a suspension in a light hydrocarbon liquid such as a light lubricating oil having a Saybolt viscosity of about 75 to 100 seconds at 100° F., or even

5 lighter hydrocarbon vehicles such as refined kerosene or naphtha. A suitable material which is available commercially contains about 10% of colloidal graphite and 90% of a light lubricating oil such as indicated above.

The low boiling solvent, preferably a hydrocarbon oil, which constitutes the major proportion (usually more than 60%) of the lubricant of this invention, should be below the lubricating oil boiling range. It may be a mineral seal oil which has a boiling range of about 510 to 670° F. or a kerosene which has a boiling range of about 375 to 510° F., or various refined naphthas, e. g., those having boiling ranges such as from 300 to 380° F., 220 to 310° F., 160 to 230° F., or even still lower boiling such as 140 to 210° F. The primary purpose of using such a low-boiling oil is that it evaporates at high temperature without formation of varnish or tar, or eventual carbonization.

15 The viscosity-increasing, linear aliphatic polymer should preferably be a high molecular weight, linear type, substantially saturated polymer of an unsaturated aliphatic hydrocarbon, which polymer, upon heating, depolymerizes without carbonization or tar formation. As this constituent, it is preferred to use a polyisobutylene having an average molecular weight above 800 and preferably above 2,000, and for many applications of the invention it is preferred to use a still higher molecular weight polymer such as the plastic solid type having a molecular weight above 30,000, e. g., 60,000, 80,000, 100,000, etc. Other polymerized iso-olefins having similar characteristics may be used, for instance, polymerized isoamylenes, e. g., polymerized methyl 2-butene-1, etc. The amount of such polymer to be used will depend upon a number of factors such as the molecular weight of the polymer, the desired viscosity of the finished lubricant and the conditions under which the lubricant is to be used.

20 Inasmuch as the thickening effect of the polymer is directly proportional to the molecular weight, a solution having any desired viscosity can be prepared by using a large amount of low molecular weight polymer or a small amount of high molecular weight polymer or various combinations in between. Also, since there is a tendency for the relatively lower molecular weight polymers, i. e., those having a molecular weight of about 800 to 15,000 or so, to be more heat-stable than those of a much higher molecular weight, e. g., 60,000 or 80,000, etc., it may be preferable for some purposes, i. e., where long

lubricating life is desired, to use a polymer in the lower range mentioned; whereas for other purposes it may be desirable, i. e., where a short lubricating life is sufficient, perhaps because the supply may be renewed frequently and easily, to use a polymer within the higher range of molecular weight. Some examples are: (a) a 20%-solution of polyisobutylene having a molecular weight of 5,000; (b) a 2%-solution of polyisobutylene having a molecular weight of 150,000; (c) a 5%-solution of polyisobutylene having a molecular weight of about 60,000. Under some circumstances it may be desirable to use a mixture of low, medium, or high molecular weight, as for instance a mineral seal oil containing dissolved therein 2% of polyisobutylene having an average molecular weight of about 150,000 (in order to get a large increase in viscosity with a small amount of addition agent, even though the breakdown in molecular weight of this polymer may be fairly rapid), and also containing dissolved therein about 10% by weight of a polyisobutylene having an average molecular weight of about 5,000, which, owing to the relatively greater heat stability of this polymer, will extend the life of this lubricating composition over a longer period of time at the high temperature involved.

In carrying out the invention, it is apparent from the above discussion of polymers of various molecular weights, that the amount of the polymer to be used may vary over a fairly wide range (from 0.1% to 20%, or even more). If colloidal graphite or other solid lubricant is added, the amount thereof to be used should ordinarily be about 0.5-2.0% by weight based on the total lubricating composition; preferably the amount of graphite should be about 0.1-0.3%. If the colloidal graphite is added in the form of a suspension in a light oil, as for instance a 10% suspension in oil, the amount of the suspension to be used will be about 0.5-20%.

Instead of polyisobutylene, one may use other thickeners such as various isobutylene co-polymers of high molecular weight, e. g., the almost saturated isobutylene-butadiene copolymer made at temperatures below 0° C., e. g., -70° C., -80° C., etc., using as catalyst a solution of a Friedel-Crafts halide dissolved in an alkyl halide solvent, e. g.,  $\text{AlCl}_3$  in methyl chloride, and preferably in the presence of liquified propane, ethane, ethylene or other inert gas as refrigerant-diluent. Another suitable thickener is the oil-soluble, substantially saturated isobutylene-ethylene copolymer made at 100-400° C., using high pressure, e. g., 500, 1,000, or 2,000 atmospheres, preferably with addition of a small amount of oxygen.

If desired, small amounts of other addition agents may be added to the lubricating composition, as for instance 0.1 to 2 or 3% of an ester, as for example the low molecular weight alkyl ester of a fatty acid, having the property of increasing the oiliness or lubricity of the composition. Small amounts of other materials such as oxidation inhibitors, depolymerization inhibitors, extreme pressure lubricating agents, etc., may be added.

Without intending to limit the invention to the particular materials used nor to the proportions in which they were used, the following account is given of a number of industrial applications of this invention. In these tests the mineral seal oil used had a boiling range of about 510-665° F., and the polybutene had an average molecular weight of about 60,000.

The graphite suspension used contains about

10% colloidal graphite and 90% of a light lubricating oil having a viscosity of about 75-100 seconds Saybolt at 100° F., and the ester, used in some instances, was an isopropyl ester of wax oxidation acids.

The various compositions used are shown in the following table, which also indicates in certain tests the approximate temperature to which the lubricant was exposed.

10

Table I

|    |                               | Percent comp.—Test No. |      |     |      |      |
|----|-------------------------------|------------------------|------|-----|------|------|
|    |                               | 1                      | 2    | 3   | 4    | 5    |
| 15 | Polybutene                    | 7.5                    | 4.3  | 15  | 1.7  | 7.9  |
|    | Colloidal graphite suspension | 5.0                    | 2.0  | 3   | 2.0  | 2.0  |
|    | Ester                         | 1.0                    | 1.0  |     |      | 1.0  |
|    | Mineral seal oil              | 86.5                   | 92.7 | 82  | 96.3 | 89.1 |
|    | Temp. of use (°F.)            | 1,000                  | 800  | 600 | 550  | 500  |
| 20 | Method of application:        |                        |      |     |      |      |
|    | Oil can                       | x                      | x    |     |      | x    |
|    | Oil cup                       |                        |      | x   |      |      |
|    | Mechanical lubricator         |                        |      |     | x    |      |

All of the above compositions were found satisfactory, some of them being used for the lubrication of annealing oven car wheel bearings, oven conveyor chains, and kiln car roller bearings, bearings of motor-gear sets subjected to radiant heat of hot metal (as hot as 1100° F.), and bearings of elevators and conveyors handling hot coke.

In these various industrial uses, great difficulty had previously been experienced in lubricating the equipment but the compositions of this invention gave excellent results. In a number of cases, after use for a considerable time with these new lubricating compositions, the equipment was disassembled in order to examine the bearings, and invariably the latter showed no signs of carbonaceous deposits and only a thin film of colloidal graphite.

An additional practical advantage of this invention is illustrated in the case of test No. 4 where the annealing oven conveyor now rolls readily by gravity, whereas formerly (with previous lubricants) men had difficulty pushing the articles being conveyed on this conveyor. Other industrial applications were made using lubricants consisting entirely of mineral seal oil and polybutene, i. e., without any colloidal graphite or other noncombustible solid material.

Typical of such applications are the lubrication of oven conveyor bearings operating at 420° F., with oil cup application where a blend of 15% polybutene, 85% mineral seal oil was utilized; the same lubricant successfully operated on electric motor bearings at temperatures so high that it had previously been impossible to keep even high temperature soda base greases in the bearing housing. Lubrication of ejector pins and other moving hot parts of die-casting machines has been most successful with a blend of 7.5% polybutene, 1% ester, 91.5% mineral seal oil.

All of these applications are being much more successfully lubricated than with any other previously used lubricants, and show that for certain types of uses the graphite not only may be, but should be, omitted from the composition.

Since the viscosity of the solution of polymer in mineral seal oil is an important factor in obtaining the proper feeding of the lubricant to suit the various types of lubrication means, used in industry, such as referred to at the bottom of the above table, or even by hand where a thick plastic lubricant is used, the following table is given in order to show the effect of the percentage of polymer used, on the viscosity of the mineral

60

65

70

75

seal oil. (The polymer used here was a polyisobutylene having an average molecular weight of about 60,000.)

Table II

| Percent of polybutene | Viscosity (seconds Saybolt at 100° F.) of mineral seal oil solution |
|-----------------------|---------------------------------------------------------------------|
| 0                     | 40                                                                  |
| 2.0                   | 100                                                                 |
| 3.5                   | 300                                                                 |
| 5.5                   | 925                                                                 |
| 25.0                  | <sup>1</sup> Plastic mass                                           |

<sup>1</sup> Must be hand-packed.

The amount of mineral seal oil used in Table II was in all cases 100% minus the amount of polybutene used. The mineral seal oil itself had a flash point of 260-270° F. and a Saybolt viscosity of about 40 seconds at 100° F.

A still further advantage of the present invention is that these new lubricants do not run or spread appreciably at the high operating temperatures involved. Their superiority in this respect over prior art lubricants is readily demonstrated by the following simple tests:

*Test A.*—A refined petroleum lubricating oil fraction having a viscosity of exactly 100 seconds Saybolt at 100° F. when dropped onto a hot metal surface (having a temperature of 400° F. or higher) having an area of about 8 inches by 10 inches will require only about 10-12 drops to spread over the entire surface.

*Test B.*—A solution of 60,000 molecular weight polybutene in mineral seal oil having a concentration sufficient to make a solution having exactly the same viscosity, namely, 100 seconds Saybolt at 100° F., when dropped onto the same type of hot metal surface in the same quantity, i. e., about 10-12 drops, will cover only about 1 square inch of surface. In other words, in round figures, the plain mineral oil spreads over about 50 to 100 times as great an area as the mineral seal oil solution of polybutene having the same viscosity. This means that the polybutene solution forms correspondingly a 50- to 100-times thicker layer or film of lubricant on the hot metal surface, and, consequently, these polybutene solutions do not run out of the bearings like the plain mineral lubricating oils of the corresponding viscosity. Furthermore, this advantage of greater thickness of lubricant film becomes even greater when more viscous oils and solutions are compared, for instance, those having a viscosity of 300 seconds or 1,000 seconds Saybolt at 100° F.

Although the theory of the mechanism of the operation of the invention is not entirely understood, it is believed to depend partly upon the use of an operating temperature sufficiently high to cause at least partial depolymerization of the polymer. Conversely, it is believed that the polymer or thickening agent should be one which decomposes, by depolymerization or otherwise, when subjected to operating temperatures involved, and does so without leaving any substantial amount of carbonaceous residue. Furthermore, the mineral seal oil or other even more volatile solvent which appears to be necessary primarily as a vehicle or fluid medium for getting the polymer, alone or with the graphite, into place in the bearing, should be a liquid which evaporates under the operating temperatures involved, without leaving any carbonaceous, varnish-like

or tarry residue, which would either undesirably increase the resistance of the moving metal parts or would cause harmful abrasion thereof.

It is not intended that the invention be limited to any of the materials which have been mentioned merely as specific examples, nor by the specific proportions given for the sake of illustration, nor by any theory as to the mechanism of the invention, but only by the appended claims in which it is intended to claim all novelty inherent in the invention as broadly as the prior art permits.

I claim:

1. The method of lubricating hot metal surfaces which, in the absence of a lubricant, would move in contact with each other, at temperatures above about 400° F., which comprises applying to said moving metal parts a lubricant comprising a major proportion of a volatile solvent having a final boiling point below 750° F., having a viscosity below 45 seconds Saybolt at 100° F. and capable of evaporating at such high temperatures without leaving any harmful residue, said lubricant also containing a sufficient amount of an oil soluble organic thickener comprising essentially a saturated linear aliphatic polymer having a molecular weight above about 800, adapted to be decomposed at such high temperatures without leaving any substantially harmful residue, to make a solution having a viscosity of at least 100 seconds Saybolt at 100° F., the product of the percent of polymer times the molecular weight of the polymer being at least 100,000.
2. The method of lubricating hot metal surfaces which, in the absence of a lubricant, would move in contact with each other, at temperatures above about 400° F., which comprises applying to said moving metal parts a lubricant comprising a major proportion of a volatile hydrocarbon oil having a final boiling point below about 675° F. and having a viscosity below about 45 seconds Saybolt at 100° F. and capable of evaporating at such high temperatures without leaving any harmful residue, said lubricant also containing dissolved therein a thickener comprising essentially a saturated hydrocarbon polymer having a molecular weight above 800 adapted to be decomposed at such high temperatures without leaving any substantially harmful residue and having the property of greatly reducing the spreading tendency of the volatile solvent, the amount of said thickener being sufficient to make a solution having a viscosity of at least 100 seconds Saybolt at 100° F., the product of the per cent of polymer times the molecular weight of the polymer being at least 100,000.
3. The method of lubricating metal surfaces at a temperature above 400° F. which comprises applying to said moving metal parts a lubricant consisting essentially of mineral seal oil and polyisobutylene, the amount of said polyisobutylene being sufficient to make a solution having a viscosity of at least about 100 seconds Saybolt at 100° F.
4. The method of lubricating metal surfaces at temperatures above about 400° F. which comprises applying to said moving metal parts a lubricant comprising a major proportion of a hydrocarbon oil having a final boiling point below about 675° F. and having a viscosity below about 45 seconds Saybolt at 100° F., said lubricant also containing dissolved therein a sufficient amount of a saturated hydrocarbon polymer having a molecular weight above 800 to make

a hydrocarbon solution having a viscosity above 100 seconds Saybolt at 100° F., the product of the per cent of polymer times the molecular weight of the polymer being at least 100,000, and said lubricant also containing a small amount of a non-abrasive solid lubricant which is non-combustible at temperatures up to about 2500° F.

5. The method of lubricating hot metal surfaces which, in the absence of a lubricant, would move in contact with each other at temperatures above about 400° F., which comprises applying to said moving metal parts a lubricant consisting essentially of a major proportion of mineral seal oil, about 0.1%-20% of polyisobutylene having a molecular weight above 800, the amount of said polymer being sufficient to make a mineral oil solution having a viscosity of at least 100 seconds Saybolt at 100° F., the product of the percent of polymer times the molecular weight of the polymer being at least 100,000, said lubricant also containing about .05% to 2.0% of colloidal graphite.

6. A high temperature lubricant for use at temperatures above about 400° F., comprising a major proportion of a volatile solvent having a final boiling point below 750° F. and capable of evaporating at said high temperatures without leaving an undesirable residue, said lubricant also containing a sufficient amount of thickener comprising essentially a saturated linear aliphatic polymer having a molecular weight above about 800, soluble in said solvent and capable of decomposing at said high temperatures without leaving any substantial harmful residue, to make a solution having a viscosity of at least 100 seconds Saybolt at 100° F., the product of the per cent of polymer times the molecular weight of the polymer being at least 100,000, and also containing a small amount of a comminuted, non-abrasive solid lubricant which is non-combustible at temperatures up to about 2500° F.

7. A high temperature lubricant for lubrication of moving metal parts at temperatures above about 400° F., which comprises at least 60% by weight of mineral seal oil, about 0.1-20% of polyisobutylene having a molecular weight above about 800, the amount of said polymer being sufficient to make a mineral oil solution having a viscosity of at least 100 seconds Saybolt at 100° F., the product of the per cent of polymer times the molecular weight of the polymer being at least 100,000, said lubricant also containing about .05%-2.0% of colloidal graphite.

8. A high temperature lubricant for use at temperatures above about 400° F. consisting essentially of a major proportion of mineral seal oil and a minor proportion of polyisobutylene having an average molecular weight above about 800, the amount of said polyisobutylene being 60

sufficient to make a solution having a viscosity of at least about 100 seconds Saybolt at 100° F.

9. A high temperature lubricant for use at temperatures above about 400° F., consisting essentially of a major proportion of mineral seal oil and dissolved therein a minor proportion of a thickener consisting of a linear aliphatic polymer having a molecular weight above 2000 and capable of decomposing at said high temperatures without leaving any substantial harmful residue, the amount of said polymer being sufficient to make a solution having a viscosity of at least about 100 seconds Saybolt at 100° F.

10. Lubricant according to claim 9 in which the arithmetic product of the per cent of polymer times the molecular weight of the polymer is at least 100,000.

11. A high temperature lubricant for use at temperatures above about 400° F., consisting essentially of about 82 to 96% by weight of mineral seal oil and about 2 to 15% by weight of polyisobutylene having a molecular weight of about 60,000.

12. Lubricant according to claim 11 also containing about 2 to 5% by weight of a colloidal graphite suspension comprising essentially about 10% by weight of graphite and about 90% by weight of a light lubricating oil.

13. A high temperature lubricant for use at temperatures above about 400° F., comprising at least 60% of a volatile solvent having a final boiling point below 750° F., a flash point of at least 260° F., a viscosity below about 45 seconds Saybolt at 100° F., and capable of evaporating at said high temperatures without leaving an undesirable residue, said lubricant also containing dissolved therein an oil-soluble saturated linear aliphatic polymer serving as thickener, having a molecular weight above 800 and capable of decomposing at said high temperatures without leaving any substantial harmful residues, in amounts sufficient to make a solution having a viscosity of at least 100 seconds Saybolt at 100° F., the arithmetic product of the per cent of polymer times the molecular weight of polymer being at least 100,000, and said total composition being capable of being heated to temperatures above 400° F. to complete dryness without leaving an undesirable residue.

14. A high temperature lubricant for use at elevated temperatures such as about 400 to 1000° F., having a viscosity of at least 100 seconds Saybolt at 100° F., consisting essentially of mineral seal oil containing about .05-2.0% of colloidal graphite and about 2 to 25% by weight of a linear substantially saturated aliphatic hydrocarbon polymer having a molecular weight above about 30,000.

DONALD L. WRIGHT.